

June 21, 1955

C. BIRDSEYE

2,711,369

PROGRESSIVE EXPLOSION PROCESS OF DEFIBRATION

Filed March 17, 1951

2 Sheets-Sheet 1



Fig. 1

Fig. 3

INVENTOR.

Clarance Birdseye.

BY

Clarence, Jenney, Witte & Hilditch.  
Attns.

June 21, 1955

**C. BIRDSEYE**

2,711,369

## PROGRESSIVE EXPLOSION PROCESS OF DEFIBRATION

Filed March 17, 1951

2 Sheets-Sheet 2



*INVENTOR.*

Clarence Birdseye.

BY

Young, Jemmy. Witter & Fielder.  
Atg

1

2,711,369

## PROGRESSIVE EXPLOSION PROCESS OF DEFIBRATION

Clarence Birdseye, Gloucester, Mass., assignor, by mesne assignments, to Process Evaluation and Development Corporation, New York, N. Y., a corporation of Delaware

Application March 17, 1951, Serial No. 216,212

8 Claims. (Cl. 92—1)

The present invention comprises an improved process for separating individual fibers, or relatively small groups or bundles of fibers, from larger units of fibrous materials such as wood chips, bark, plant stalks, or asbestos rock fragments. The process of my invention is characterized by the use of successive explosions, each of which only partially separates the fibrous material being defibrated or disintegrated, and thereby permits the use of such low pressures and temperatures as the explosive force that the fibers of the material being treated are neither seriously damaged physically nor importantly altered chemically.

The invention includes within its scope novel apparatus for carrying out my improved process. This apparatus may vary considerably in detail, but in all its embodiments is characterized by its ability and capacity to produce numerous explosions of controlled force in the product being treated while that product is passing continuously through the apparatus.

I am aware that the defibration by the explosive expansion of fluids within fibrous materials is not broadly new. But heretofore it has been the main objective of such processes to build up a pressure substantially equal throughout the entire mass of each unit of product being treated and then, by suddenly and simultaneously relieving all the pressure throughout each of the units, to separate each unit completely and instantaneously into its component fibers. To accomplish such practically simultaneous defibration or disintegration of the relatively large product units, such as papermill chips or pieces of asbestos rock, it has been necessary to bring the entire mass of each unit of material to substantially uniform temperature and/or pressure; and to accomplish sufficiently rapidly this balancing of pressure and/or temperature throughout whole units has required the use of very high pressures and temperatures within the treating apparatus. In the commercial production of "Masonite," for instance, wood chips are subjected to steam pressures of 1000 p. s. i. or more prior to explosion. The use of such steam pressures and the accompanying extremely high temperatures partly hydrolyzes wood and brings about other chemical and physical changes which it is an object of my invention to avoid.

It is the principal object of my invention to bring about defibration with a minimum of chemical or physical change other than defibration itself. In accomplishing this result I provide a process in which each fibrous unit is exposed to a minimum of effective heat and/or pressure prior to explosion. The desired objectives are accomplished by successive explosions each of a relatively mild nature and, preferably, all occurring at progressively lower pressures and/or temperatures.

By the process of my invention progressive—as definitely opposed to simultaneous—defibration of each unit of the product under treatment may be brought about by specifically different procedures best carried out in apparatus of somewhat different design.

Going more into detail and dealing with spruce wood

2

chips by way of illustration, it is proposed to deliver the chips after they come from the "hog" or chopper in preheated condition to a pressure space, such as that formed between the pistons in the cylinder of a continuous pressure cooker of the general type of that disclosed in U. S. Patent No. 2,403,871, McBean. Each pressure space or compartment between two spaced pistons is filled to only about 25% capacity, thus allowing space for expansion of the product during successive explosions. As soon as each compartment is loaded and has passed into the cylinder steam is admitted through a port in the cylinder wall to bring the pressure in the compartment to approximately 50 p. s. i. (approximately 297° F.). Some of the steam will be condensed and moisture and heat will immediately begin to penetrate toward the interior of each chip. Then as each compartment passes forwardly over the next port in the cylinder wall, additional steam is admitted to the compartments one after another till the pressure within them is brought to about 100 p. s. i. (about 338° F.), thus causing penetration of moisture, heat and pressure further toward the center of each chip. Again, as each compartment progresses past the next (third) port in the cylinder wall, steam is admitted to a pressure of 200 p. s. i. (about 387° F.); and penetration of heat, moisture and pressure continues into all the deeper portions of the chips. Finally, as the several compartments pass over the final steam inlet port, pressure within the chamber is raised to 300 p. s. i. (about 422° F.).

By the time the atmosphere in each compartment has reached this final pressure the smaller chips and particles of wood in that compartment will have been equalized as to temperature, moisture and pressure throughout their masses; but the larger chips will not yet have become heated at their centers to the same temperature as their exteriors. Inasmuch as the rate of penetration of moisture, heat and pressure into each fragment of wood is dependent on the time and temperature factors, the penetration rate can be regulated to accomplish any desired degree of penetration merely by varying either or both the speed at which the compartments are advanced through the cylinder or the steam pressures admitted to the compartments as they pass over the several steam inlet ports.

Immediately—or at least very soon—after the chips in any compartment have been subjected to the desired conditions of heat and steam pressure, that compartment in advancing through the cylinder, travels past a series of decompression ports, at each of which the pressure in the compartment is explosively lowered to any desired point pressure; and I have found that with spruce chips the optimum decompression rate should be about 100 p. s. i. per step.

Thus at the first decompression port the pressure in each successive chamber or compartment is suddenly dropped from 300 p. s. i. to 200 p. s. i., preferably by injecting into the compartments, through a port in the cylinder, the necessary amount of a relatively cold liquid, such as a spray of water or of one of the chemical digestants commonly used in pulp making. Alternatively, a suitable pop-valve in the upper part of the cylinder may be used to relieve pressures, or any other suitable pressure-reduction means may be employed.

As the result of the first sudden release of pressure in each chamber all of the smaller chips, which had previously become pressure- and temperature-stabilized throughout their masses, will be instantly entirely defibrated or disintegrated, and the larger chips, which have up to that time been only partly heat-penetrated, will be explosively defibrated as to those outer parts of their mass which have become sufficiently heat- and pressure-penetrated. This step thus exposes fresh lay-

ers of fibre in the larger chips to the direct action of steam or caustic vapor.

As the result of the second of these explosive reductions of pressure (that from 200 p. s. i. to 100 p. s. i.) some of the residual chips will be entirely, and others partially disintegrated. In the meantime, further heat penetration will be occurring in the freshly exposed layers of fibre in the still unexploded chips.

At the time of the third explosive pressure drop (that from 100 p. s. i. to atmospheric) the desired disintegration or defibration of all the product units in each chamber will be completed, and thereafter the now fibrous mass will be carried to the exit from the cylinder, and will be in form for any further desired treatment.

Under the above conditions I find that spruce chips of the size and nature commonly used in paper making require from about 30 to 60 seconds to pass through the entire length of the cylindrical cooker—the exact time required depending upon the diameter and length of the cylinder, the amount and maximum size of chips loaded into each pressure space or compartment, and the temperatures and pressures employed.

In the application of my process as described above no effort is made to remove from the fibers the lignin, terpenes or other non-cellulosic materials surrounding them. That can be done subsequently by any of several well-known commercial processes, or in any of several equally well-known commercial types of equipment designed for that purpose.

In carrying out my improved process the chips will be more or less moist or wet when fed into the continuous cooker, and a certain amount of moisture will be added to the chips each time steam is fed into the compartments during the pressure-raising phase of the process. On the other hand, if the subsequent pressure-lowering operations are accomplished by passing the chips under pop-valves to reduce progressively the pressures in the several compartments considerable moisture will be carried out of the cylinder as each explosive pressure-reduction is accomplished. The masses of fibers will therefore become somewhat dry and quite fluffy as the contents of each compartment is finally discharged from the cooker. If, on the contrary, the several pressure reductions within the cooker are accomplished by the addition of a cold water spray or other liquid to the compartments the product finally discharged from the cooker will be a fluid mixture of liquid and solids, which may subsequently be separated in any desired manner, as for instance, by means of a Fourdrinier belt.

"Digestion" (i. e. separation of cellulosic and non-cellulosic materials) can, by a modification of my process, be accomplished simultaneously with the heating and exploding steps. One way in which digestion of the chips may be thus accomplished is by injecting, instead of steam, a caustic digestive fluid such as a solution of caustic soda or sodium sulphite into the cylinders under pressures of respectively 100, 200 and 300 p. s. i., and then explosively reducing the pressures within each chamber to 200, 100 and atmospheric by passing the chambers successively under properly regulated pop-valves. Thereafter, the cellulose fibers and the digestive fluid can be separated by any of several well-known commercial means—e. g. centrifuges, vibrating screens, or Fourdrinier belts.

Although I have hereinabove suggested the use of a modified "McBean type" continuous cooker, with heat and pressure supplied by the injection of either steam or a hot digestive fluid under pressure, I do not wish to be limited to such means, for my process of defibration by repeated explosions can be carried out in any suitable apparatus and with any available means of bringing about the successive explosions which characterize my process.

The advantages of my present process, as compared with such short-time-high-pressure-single-explosion methods as those disclosed in Mason's U. S. patents (above identified) are numerous. As applied to the production of paper pulp: the enormous pressures and extremely high temperatures employed in the Mason process hydrolyze some of the non-cellulosic constituents of the wood, and shorten and split the individual cellulose fibers. On the other hand, the lower pressures and temperatures of my improved process—made possible by progressive heat penetration and repeated less violent explosions—present certain definite advantages; and the gradual build-up and step-down of pressures at opposite ends of a cylindrical cooker greatly simplify the construction and operation of that type of apparatus. This could not be used at all if pressures as high as 1000 p. s. i. were necessary within it and throughout its length. As applied to such inorganic fibrous or laminated materials as asbestos rock and mica, my multiple, comparatively mild explosions have the great advantage of adequately fractionating relatively large units almost wholly along natural cleavage lines and with a minimum of breakage across the grain of the fibers or laminations.

The features and advantages of my improved process will best be understood and appreciated from the following description of apparatus for carrying it out as illustrated in the accompanying drawings in which:

Figs. 1 and 2 are complementary views in elevation, partly in longitudinal section, of the apparatus, and

Fig. 3 is a diagrammatic view illustrating the general condition of the product in successive stages of the process.

As herein shown the apparatus includes an elongated, metal pressure cylinder 10 horizontally disposed and provided throughout a part of its length with a steam jacket 11. An opening is provided near the intake end for a feed hopper 12 through which raw material, for example pre-heated wood chips, may be introduced into the cylinder.

A series of compartments or chambers is formed within the cylinder 10 by pistons 13 securely affixed to a sprocket chain 14 in uniform spacing. The sprocket chain runs over sprocket wheels 15 and 16 and, of these, the wheel 16 may be driven from any convenient source of power to draw the pistons from left to right through the length of the cylinder in pressure tight relation and then return them freely from right to left outside the cylinder. In a cylinder having an effective length of 10 feet the pistons may be advanced at a rate of 10 to 20 feet per minute depending on the character of the raw material being treated.

The cylinder is provided in the portion shown in Fig. 1 with steam connections comprising pipes 17, 18 and 19 which enter the lower side of the cylinder in uniform spacing corresponding approximately to the spacing of the pistons 13. Substantially opposite each pipe in the cylinder is provided a pressure gauge 20. Each adjacent pair of pistons 13 forms a compartment, one of which in Fig. 1 is shown as being in communication with the pipe 17 by which it may be supplied with steam or vaporized caustic soda solution at 100 pounds gauge pressure, for example. As these pistons are advanced the compartment is brought successively into communication with the pipe 18 supplying steam at 200 pounds and then the pipe 19 supplying steam at 300 pounds. As the charge of wood chips is advanced in this manner the chips become permeated wholly or partly with steam or caustic solution at the pressures indicated and are now ready to be subjected to a series of defibrating explosions.

The cylinder is provided in the portion shown in Fig. 2 with connections 21, 22 and 23 to individual explosion chambers each controlled by an adjustable pressure-relief valve as indicated conventionally in the drawings. These connections are spaced to correspond approximately with the spacing of the pistons 13 and may be separated from

the steam connections by any desirable length in the tube 10 through which the charge of chips may be conveyed while maintained under maximum steam pressure. In the illustrated apparatus it may be assumed that the pressure-relief valve in the connection 21 is set at 200 pounds. Consequently when the foremost cylinder defining the compartment passes the outlet of the connection 21, the pressure therein is explosively dropped from 300 to 200 pounds and the effect upon the chips is to defibrate and disintegrate at least the surface layers of the chips in the charge.

As the piston-defined compartment is advanced the chips remain under 200 pounds steam pressure and if the chips have not been completely permeated hitherto by steam at that pressure, the newly exposed layers of fibre in the chips are quickly brought to that condition. When the connection 22 is reached the pressure in the compartment is again explosively reduced this time from 200 to 100 pounds and again the exposed portion of the chips is defibrated and disintegrated. When the pistons reach the final connection 23 a third explosive reduction in pressure takes place, this time from 100 pounds to atmospheric pressure, and in this final stage the chips are totally reduced to their constituent fibres.

Fig. 3 illustrates diagrammatically the three steps of the process above described. A typical chip 30 is indicated at the left-hand side of the figure as it is introduced into the pressure cylinder and it may be assumed that the chip 31 represents the condition of the same chip after it has been subjected to the first explosive reduction in pressure. The fibres constituting the surface portion of the chip have been loosened and separated from the body of the chip. The core of the chip and the fibres separated therefrom when subjected to explosive pressure reduction from 200 to 100 pounds are represented at 32. And finally, the group of disintegrated fibres 33 represents the ultimate condition of the original chip.

After the final explosive reduction in pressure and a complete defibration of the chips the fibres are discharged from the right-hand end of the cylinder 10 and are directed through a discharge hopper 24 to a wire mesh conveyer 25 horizontally disposed and adapted to remove the fibres from the apparatus while permitting intrained liquid to drain away to a tank 26 disposed beneath the conveyer. When a hot caustic solution is used, it will carry with it the non-cellulosic material dissolved from the chips.

The connections 21—23 each include a pressure relief valve as already explained, and are herein shown as leading upwardly to chambers 27 which act as mufflers and also serve to retain stray fibres that may be blown out of the pressure tube. If desired the pistons 13 may be enclosed throughout a portion of their return run and thus the capacity of the apparatus correspondingly increased.

While the exact pressures employed are of course of secondary importance, they must in all cases be sufficient to cause explosive disintegration of the fibrous product when suddenly reduced or released at successive stations in the process.

Having thus disclosed my invention and described in detail an illustrative manner of carrying it out, I claim as new and desire to secure by Letters Patent:

1. In a process of reducing fibrous material to its constituent fibres, the steps of confining a predetermined charge of the material under vapor pressure of a hot caustic solution at a pressure of approximately 300 p. s. i., then advancing the compressed charge to a series of decompression stations and explosively reducing the vapor pressure of the charge first to approximately 200 p. s. i., then to 100 p. s. i., thus exposing fresh layers of fibres at each step to direct action of hot caustic vapor, and finally to atmospheric pressure.

2. In a process of defibrating fibrous cellulose-yielding material, the steps of building up in an intermittent and

progressive manner a gaseous pressure of not less than 100 p. s. i. within fragments of the material, and then intermittently reducing the said gaseous pressure thereby subjecting the fragments to a series of disintegrating explosions at progressively decreasing pressures and so progressively exposing fresh layers of fibre directly to gaseous pressure.

3. In a process of defibrating wooden chips, the steps of enclosing a collection of chips in a pressure space, subjecting the collection to internal gaseous pressure greater than atmospheric, explosively disintegrating the chips by a series of steps at progressively decreasing pressures thus removing surface fibres from each chip and exposing fresh layers of fibre directly to gaseous pressure, and subjecting the residual chips to moisture at all intermediate stages while the said chips are contained in the original pressure space.

4. In a process of reducing wood chips to their constituent fibres, the step of enclosing in a compression space a collection of chips of different sizes, subjecting the collection to internal gaseous pressure greater than atmospheric, and reducing the pressure progressively in a series of explosive steps at progressively decreasing pressures thereby converting some of the smaller chips to loose fibres and progressively removing surface fibres from the larger chips thus exposing fresh layers of fibre directly to gaseous pressure.

5. In a process of reducing fibrous chips to their constituent fibres, the steps of enclosing the chips in a pressure chamber in a predetermined location, moving the enclosed chips progressively in series from station to station, subjecting them to intermittently increasing steam pressures at certain stations, and subjecting them to explosions under progressively decreasing pressures at stations later in the series thereby successively exposing fresh layers of fibre in the chips to steam pressure.

6. In a process of reducing fibrous cellulose-yielding material to its constituent fibres, the steps of subjecting the material to predetermined initial pressure of vapor of a digestant fluid at approximately 300 p. s. i., and then explosively reducing the internal pressure of the material in a series of steps of decreasing pressure, exposing fresh layers of fibre directly to vapor pressure at each step and maintaining the material between the said steps under internal pressure and in contact with the said digestant fluid.

7. In a process of reducing fibrous material to its constituent fibres, the steps of confining a predetermined charge of the material, progressively building up an increasing internal fluid pressure in the charge of approximately 300 p. s. i., and then progressively and explosively reducing said pressure in a step by step manner thus progressively exposing fresh layers of the material directly to fluid pressure.

8. In the defibration of pieces of fibrous vegetable material, the process comprising the steps of subjecting the pieces to a hot caustic solution at greater than atmospheric pressure thereby dissolving the non-cellulosic material from between the cells of the pieces, then explosively disintegrating the pieces in a series of steps at progressively decreasing pressures and thereby separating at least the surface cells of the pieces and exposing fresh layers of fibre directly to the action of hot caustic vapor, and then separating the loose cells from the caustic solution.

65 References Cited in the file of this patent

UNITED STATES PATENTS

|              |                        |               |
|--------------|------------------------|---------------|
| 47,539       | Fuller et al. -----    | May 2, 1865   |
| 530,635      | Blackman -----         | Dec. 11, 1894 |
| 982,379      | Marshall -----         | Jan. 24, 1911 |
| 1,383,370    | Bancroft -----         | July 5, 1921  |
| 1,632,467    | Fish -----             | June 14, 1927 |
| 1,872,996    | Mason -----            | Aug. 23, 1932 |
| 2,007,348    | Scharmann et al. ----- | July 9, 1935  |
| 2,386,401    | Joyce -----            | Oct. 9, 1945  |
| 70 2,403,871 | McBean -----           | July 9, 1946  |